

3,463,621

## ALLOYS OF SINTERED CARBIDES

Richard Kieffer, Vienna, Austria, assignor to Societe des Poudres Metalliques et des Alliages Speciaux Ugine-Carbone, Paris, France, a corporation of France  
No Drawing. Filed June 19, 1968, Ser. No. 738,137  
Claims priority, application Austria, June 20, 1967,

A 5,750/67

Int. Cl. B22f 3/10

U.S. Cl. 29—182.7

11 Claims

## ABSTRACT OF THE DISCLOSURE

An improved sintered hard metal alloy comprising 4 to 15 percent of at least one metal selected from the group consisting of iron, nickel and cobalt, 0.5 to 75 percent titanium carbide, 3 to 40 percent columbium carbide-hafnium carbide and the balance tungsten carbide. A small amount (0.1 to 0.5 percent) of vanadium carbide may be included.

My invention relates to sintered hard metal alloys and, in particular, to sintered hard metal alloys used in fabricating tools for machining materials to produce long or short chips.

In the past, sintered hard metals used in machining materials that produce short chips were comprised of tungsten carbide and cobalt to which small quantities (at least 3 percent) of additional carbides such as titanium carbide, tantalum carbide, columbium carbide or vanadium carbide were frequently added. For machining materials that produce long chips, tungsten carbide-titanium carbide alloys were used in Europe and tungsten carbide-tantalum carbide alloys were used in the United States. More recently, it has become common practice to utilize an alloy of tungsten carbide-titanium carbide-tantalum carbide and cobalt. These alloys contain from 10 to 15 percent titanium carbide plus tantalum carbide for machining soft steels and cast steels, and from 15 to 30 percent titanium carbide plus tantalum carbide for machining harder steels. For finished machining and high cutting speeds, these alloys contain from 30 to 50 percent or more titanium carbide and tantalum carbide. For finished machining and high cutting speeds, alloys with titanium carbide contents of 70 percent have been used. (All percentages referred to herein are percent by weight.)

It is a well-known fact that tantalum carbide increases the heat resistance of the tungsten carbide-titanium carbide-cobalt alloys as well as their strength. This is achieved even though tantalum carbide is a relatively soft carbide, having a Vickers hardness of 1500 to 1600, as compared to tungsten carbide and titanium carbide which have Vickers hardness of 2200 to 2400 and 3000, respectively. Attempts have been made to substitute equal amounts of columbium carbide for tantalum carbide, since it has a Vickers hardness of 2200 to 2400. However, it has been possible to replace only 30 percent of the tantalum carbide with the columbium carbide, since any larger addition causes embrittlement of the alloy. Attempts have also been made to substitute hafnium carbide for tantalum carbide (see "Hartmetalle" by Kieffer and Benesovsky) which have been successful.

This invention provides novel sintered hard metal alloys which can be used in fabricating tools for machining materials that produce both long and short chips. The invention also encompasses a method of making the alloys and tools fabricated from the alloys. The alloys of my invention comprise from 4 to 15 percent of at least one metal belonging to the iron group consisting of iron, nickel and cobalt, but preferably cobalt, 0.5 to 75 percent titani-

um carbide, 3 to 40 percent columbium carbide and hafnium carbide preferably as a mixed crystal and the balance tungsten carbide. The alloy may also contain up to 0.5 percent vanadium carbide and possibly a small percentage of tantalum carbide, which will generally be in the columbium carbide-hafnium carbide mixed crystal. Preferably, however, the alloy contains 6 to 11 percent of at least one metal belonging to the iron group consisting of iron, nickel and cobalt, but preferably cobalt, 5 to 40 percent titanium carbide, and 5 to 20 percent columbium carbide-hafnium carbide as mixed crystals or in solid solution. If vanadium carbide is included, it is preferably between 0.2 and 0.3 percent. The tantalum carbide will generally not exceed 3 percent.

By replacing the tantalum carbide with columbium carbide-hafnium carbide in tungsten carbide-titanium carbide-tantalum carbide-cobalt alloys, it has been possible to increase the hardness or the bending strength of the alloy, and at times, to increase both of these properties. These results are contrary to those to be expected in that both columbium carbide and hafnium carbide are harder than pure tantalum carbide or tantalum carbide containing small amounts of columbium carbide.

Alloys producing particularly good machining performance are those in which the amount of hafnium carbide is approximately  $\frac{1}{5}$  to 3 times that of the columbium carbide (i.e., HfC is 20 to 75 percent of the mixed crystal). Furthermore, it is often preferable that the hafnium carbide be  $\frac{1}{5}$  to 1 times the columbium carbide (HfC is 20 to 50 percent of the mixed crystal). In a long series of tests it has been shown that particularly good cutting metal alloys were produced which were superior to the well-known alloys with tantalum carbide.

The manufacture of the alloys is advantageous since the costly separation of columbium and tantalum is not required. It is possible to use columbium minerals having a low tantalum content, such as  $\frac{1}{10}$  to  $\frac{2}{5}$  of the columbium content, for the direct manufacture of columbium carbide, since the presence of corresponding amounts of tantalum carbide in the columbium carbide does not alter the properties of the alloys of the invention. Further, it is also possible to use large amounts of columbium acid containing small amounts of tantalum which arise in the separation of columbium from tantalum and in the enrichment of tantalum. These products, which up until now have served almost exclusively only in the manufacture of ferrocolumbium, therefore, have a new and novel market.

The columbium carbide-hafnium carbide solid solutions may be added, at least in part, in the form of ternary columbium carbide-hafnium carbide-tungsten carbide mixed crystals or columbium carbide-hafnium carbide-titanium carbide mixed crystals, or in the form of quaternary columbium carbide-hafnium carbide-titanium carbide-tungsten carbide mixed crystals. At the time of the preparation of these mixed crystals, 20 to 40 percent of the tungsten carbide and/or the titanium carbide can be added. Therefore, significant self-purification can be obtained in the usual way as far as oxygen and nitrogen are concerned. Such mixed crystals have, for example, the following composition:

50 parts NbC, 50 parts HfC, 40 parts WC,  
or 70 parts NbC, 30 parts HfC, 20 parts WC,  
or 100 parts TiC, 40 parts WC, 20 parts NbC, 40 parts HfC.

It has also been proven practical to add 0.1 to 0.5 percent, and preferably 0.2 to 0.3 percent vanadium carbide to the basic alloy.

In the preparation of alloys of my invention, I prefer to add columbium carbides and hafnium carbides, and

possibly tungsten carbides and titanium carbides, wholly or in part, in the form of grains the size of which is less than 1 micron, and preferably less than 0.1 micron.

The following compositions illustrate alloys of my invention which are intended for machining materials producing long chips:

| TiC<br>(percent<br>by wt.) | NbC<br>(percent<br>by wt.) | HfC<br>(percent<br>by wt.) | TaC<br>(percent<br>by wt.) | Co<br>(percent<br>by wt.) | WC<br>(percent<br>by wt.) |
|----------------------------|----------------------------|----------------------------|----------------------------|---------------------------|---------------------------|
| 6                          | 3                          | 3                          | -----                      | 10                        | Remainder.                |
| 16                         | 7                          | 3                          | -----                      | 8                         | Do.                       |
| 16                         | 5                          | 3                          | 2                          | 7                         | Do.                       |
| 18                         | 4                          | 6                          | -----                      | 9                         | Do.                       |
| 25                         | 5                          | 5                          | -----                      | 9                         | Do.                       |
| 40                         | 5                          | 3                          | 2                          | 7                         | Do.                       |

The following compositions are typical of alloys of my invention intended for machining materials producing short chips:

| TiC<br>(percent<br>by wt.) | NbC<br>(percent<br>by wt.) | HfC<br>(percent<br>by wt.) | TaC<br>(percent<br>by wt.) | Co<br>(percent<br>by wt.) | WC<br>(percent<br>by wt.) |
|----------------------------|----------------------------|----------------------------|----------------------------|---------------------------|---------------------------|
| 0.5                        | 2                          | 1.5                        | 0.5                        | 6                         | Remainder.                |
| 1                          | 1                          | 2                          | -----                      | 5                         | Do.                       |

The following table shows the bending strength and hardness of the hard metal alloys produced according to my invention as compared with standard tungsten carbide-titanium carbide-tantalum carbide (columbium carbide) cobalt alloys. As is shown, it is evident that my alloys exhibit superiority with respect to the bending and 30 hardening strength of the metal alloys.

TABLE 1

|                                   | TiC | Co | WC   | NbC(TaC)+HfC   | Bending<br>strength,<br>kg./mm. <sup>2</sup> | HV/60<br>Vickers<br>hardness,<br>kg./mm. <sup>2</sup> |
|-----------------------------------|-----|----|------|----------------|----------------------------------------------|-------------------------------------------------------|
| Known alloys.....                 | 16  | 7  | Rest | 8 TaC          | 115-125                                      | 1,500-1,600                                           |
|                                   | 16  | 7  | do   | 6 TaC+2NbC     | 110-120                                      | 1,550-1,650                                           |
| Alloys of the in-<br>vention..... | 16  | 7  | do   | 6NbC+2 HfC     | 120-130                                      | 1,650-1,750                                           |
|                                   | 16  | 7  | do   | 4NbC+2TaC+2HfC | 120-130                                      | 1,550-1,650                                           |
|                                   | 16  | 7  | do   | 4NbC+4 HfC     | 140-150                                      | 1,600-1,700                                           |
|                                   | 16  | 7  | do   | 2NbC+6 HfC     | 130-140                                      | 1,600-1,700                                           |

Slight improvements in the hardness and cutting content 45 can be obtained for the tungsten carbide-titanium carbide-columbium carbide-hafnium carbide alloys of my invention by the addition of from 0.1 to 0.5 percent vanadium carbide. The addition of vanadium carbide is more effective when a particularly fine columbium carbide with a grain size of less than 1 micron is used, particularly, less than 0.1 micron. The two compositions below are examples of alloys of this invention of a very fine grain size containing vanadium carbide:

| TiC<br>(percent<br>by wt.) | NbC<br>(percent<br>by wt.) | HfC<br>(percent<br>by wt.) | VC<br>(percent<br>by wt.) | Co<br>(percent<br>by wt.) | WC<br>(percent<br>by wt.) |
|----------------------------|----------------------------|----------------------------|---------------------------|---------------------------|---------------------------|
| 5                          | 3                          | 2                          | 0.2                       | 11                        | Remainder.                |
| 12                         | 8                          | 4                          | 0.2                       | 8.5                       | Do.                       |

While I have described certain preferred embodiments of my invention, it should be understood that it may otherwise be embedded within the scope of the appended claims.

I claim:

1. A sintered carbide alloy consisting essentially of 5

to 15 percent of at least one metal selected from the group consisting of iron, nickel and cobalt, 0.5 to 75 percent titanium carbide, 3 to 40 percent columbium carbide-hafnium carbide mixed crystal, up to 0.5 percent vanadium carbide, and the balance tungsten carbide and minor amounts of tantalum carbide and incidental impurities.

2. An alloy as set forth in claim 1 wherein the ratio of hafnium carbide to columbium carbide is 1/5 to 3.

3. An alloy as set forth in claim 1 in which the tantalum carbide is no greater than 2/5 the amount of columbium carbide.

4. An alloy as set forth in claim 1 having 4 to 15 percent cobalt.

5. A sintered carbide alloy consisting essentially of 15 to 11 percent of at least one metal selected from the group consisting of iron, nickel and cobalt, 5 to 40 percent titanium carbide, 5 to 20 percent hafnium carbide-columbium carbide mixed crystal, and the balance of said alloy tungsten carbide.

20 6. An alloy as set forth in claim 5 including 0.2 to 0.3 percent vanadium carbide.

7. An alloy as set forth in claim 5 wherein said hafnium carbide-columbium carbide mixed crystal comprises from 20 to 50 percent hafnium carbide.

8. An alloy as set forth in claim 6 including up to 3 percent tantalum carbide.

9. A sintered carbide alloy consisting essentially of 6 to 11 percent cobalt, 5 to 40 percent titanium carbide, 5 to 20 percent columbium carbide-hafnium carbide-tantalum carbide mixed crystal, and the balance tungsten carbide.

30

10. An alloy as set forth in claim 9 including 0.2 to 0.3 percent vanadium carbide.

11. In a sintered hard metal alloy consisting essentially of tungsten carbide, titanium carbide and at least one metal selected from the group consisting of iron, nickel and cobalt, the improvement comprising the addition of 50 3 to 40 percent columbium carbide-hafnium carbide mixed crystal.

#### References Cited

#### UNITED STATES PATENTS

|    |           |        |               |       |          |
|----|-----------|--------|---------------|-------|----------|
| 55 | 2,188,983 | 2/1940 | Padowicz      | ----- | 29—182.7 |
|    | 2,198,343 | 4/1940 | Kieffer       | ----- | 29—182.7 |
|    | 2,899,739 | 8/1959 | Ohlsson       | ----- | 29—182.7 |
|    | 2,924,875 | 2/1960 | Gisner et al. | ----- | 75—203 X |
| 60 | 3,245,763 | 4/1966 | Ohlsson       | ----- | 29—182.7 |

BENJAMIN R. PADGETT, Primary Examiner

ARTHUR J. STEINER, Assistant Examiner

65 U.S. CL. X.R.  
75—203